

March 19, 1957

G. A. MARSH

2,786,021

## METHOD FOR OBTAINING CORROSION RATE OF METALS

Filed April 21, 1953



**INVENTOR.**

BY GLENN A. MARSH

Edward H. Lang

**ATTORNEY**

2,786,021

**METHOD FOR OBTAINING CORROSION RATE OF METALS**

Glenn A. Marsh, Crystal Lake, Ill., assigner to The Pure Oil Company, Chicago, Ill., a corporation of Ohio

Application April 21, 1953, Serial No. 350,150

7 Claims. (Cl. 204—1)

This invention relates to the use of an electrochemical technique in the study of corrosion processes. It is more specifically concerned with correlating the polarization characteristics of metals with the corrosion rate of said metals.

The many complex and heterogeneous variables which may be involved in corrosion reactions make the investigation of corrosion problems very difficult. Although various attempts have been made to simulate corrosive environments and study the effect of these environments under conditions in which the rates of corrosion reactions would be accelerated by increasing the intensity of the variables involved, as a general rule the results of these tests do not correlate very readily with actual field data. As a result, the time honored technique of exposing various metallic materials of construction to actual conditions under which the metals are to be used has provided information upon which the most reliance may be placed. This technique has obvious disadvantages, such as the relatively long periods of time required to obtain sufficient information and the limitations in the technique due to the inability to vary slightly the environmental conditions under which the metallic materials of construction are to be employed. The most desirable technique would be an accelerated process which could be carried out either in the laboratory or in the field and provide sufficient information upon which the solution to engineering problems, occurring due to corrosion, could be predicated. In a copending application, Serial Number 328,779, filed December 30, 1952, there is described a polarization envelope technique which is a rapid qualitative or, at best, a semi-quantitative method for predicting the effect of electrochemical corrosion on metallic materials of construction. It has now been found that corrosion rate of metals may be quantitatively predicted. Thus, by means of the techniques which I have discovered, qualitative and quantitative investigations of electrochemical corrosion can be made.

It is therefore an object of this invention to provide an accelerated method for quantitatively determining the effect of electrochemical corrosion by means of a rapid technique which provides reproducible results. It is a further object of this invention to correlate quantitatively the effect of electrochemical polarization with corrosion rate. Another object of this invention is to provide an electronic apparatus which may be employed in carrying out investigations of the corrosion rate of metallic materials of construction exposed to electrolytic corrosive environments.

Figure 1 is a schematic diagram illustrating the essential elements of the apparatus which may be employed in carrying out this invention.

Figure 2 is a graphical presentation of the depolarization data obtained by using the apparatus shown in Figure 1 for investigating the rate of corrosion of steel in contact with an aerated brine solution containing no corrosion inhibitor. This type of curve is hereinafter referred to as the depolarization-time curve.

It is well known that corrosion of metals occurs by either direct chemical action or electrochemical action between the metals and their environment. Whereas the first type of corrosion is effected by direct chemical attack and does not require the presence of moisture, the second type of corrosion requires the presence of moisture in the corrosive environment to produce a galvanic process. In this type of corrosion there is consumed chemical energy with the production of electrical energy. It therefore should be apparent that a knowledge of the electrochemical characteristics of corrosion cells would be useful in obtaining information as to the corrosibility of various substances. The prior art does disclose the use of electrochemical techniques as a means for predicting corrosion behavior and in general these techniques have used, as a criterion, the polarization characteristics of metallic materials of construction. However none of these techniques has been used successfully in rapid qualitative and quantitative methods for investigating corrosibility and rate of corrosion, whereby results may be obtained in a matter of several minutes.

Polarization has been defined as the stoppage of the voltaic current from an electrolytic cell due to the accumulation of dissociation products at the electrodes and it is a measure of the irreversibility of an electrolytic process. Polarization may be observed by measuring the potential of an electrode as referred to a reference electrode while current is passing through the electrode with the electrode immersed in an electrolyte. The products formed at the electrode surface cause the electrode potential to change. If the electrode potential changes during the polarization in a negative direction, the polarization is cathodic. Similarly if the electrode potential changes in a positive direction, the polarization is anodic. Removal of the polarization products by either dissolving or diffusing away causes the electrode to be depolarized and the electrode potential returns to its normal electrode potential. The term "normal potential" is intended to designate the non-thermodynamic potential of the metal in the corroding environment. It has been found that by correlating time with the depolarization which occurs subsequent to the polarization produced by an instantaneous discharge of current, it is possible to produce rapidly a relative potential-time curve which may be employed in corrosion studies.

Although the production of cathodic and anodic depolarization-time curves are known electrochemical techniques, the separate cathodic and anodic depolarization effects occurring after an instantaneous discharge of current have never been studied in conjunction with each other to provide information which can be employed in corrosion studies prior to the polarization envelope technique described in my above-mentioned application. In further applying these phenomena to the study of corrosion, I have found that if the separate anodic and cathodic depolarization-time curves are simultaneously produced after an initial polarization is effected by means of an instantaneous discharge of current of sufficient intensity, and the respective variations in electrode potential occurring during the anodic and cathodic depolarization are algebraically added, the results may be graphically recorded by correlating the change in potential with time to produce a composite curve showing the net variation in potential occurring during concurrent anodic and cathodic depolarization. From this curve an empirical quantitative relationship between corrosion rate and polarization can be derived.

In investigating corrosion rate by means of this technique, the apparatus shown schematically in Figure 1 is used. This apparatus consists essentially of a power source of high voltage direct current 10, which is used to charge the capacitor 11 in a current discharge mechanism 12,

a sensitive polarization detector 13, and a polarization meter 14. Cell 15 is a receptacle which is adapted to contain an electrolytic corrosive solution to which the metallic material of construction being investigated is exposed. Test electrodes 16 and 17 are disposed within cell 15 and immersed in the electrolyte to form a simple galvanic cell. The test electrodes, which are substantially identical in size, are prepared from the metal which is being studied. This cell is then connected in parallel between the current discharge mechanism 12 and the polarization detector 13. The apparatus, as shown schematically in Figure 1, represents the simplest form of a suitable apparatus. However the device may be made more flexible in its operation by providing a bank of capacitors and suitable switches and relays in the current discharge mechanism which, as shown, consists simply of a double pole-double throw switch. Thus, in one preferred form, by means of a relay, the charged capacitor is permitted to discharge instantaneously across the two metallic electrodes 16 and 17 of the cell 15. Although the capacitor discharge mechanism shown in Figure 1 of the accompanying drawing, as well as the aforementioned modifications of this mechanism, incorporates a capacitor for effecting a brief discharge of direct current through the electrodes 16 and 17 in cell 15, it is also within the scope of this invention to employ any other suitable means whereby a direct current may be briefly passed through the said electrodes. For example, it is possible to achieve this objective by simply connecting across the electrodes a source of high voltage direct current and, by means of a mechanical or electrical relay incorporated into the power source, apply the direct current produced from the power source 10 to the electrodes 16 and 17. The time interval during which the direct current from an external source is passed through the circuit to effect the measurable polarization of the test electrodes is the time that it takes for a capacitor or other equivalent source of high voltage direct current that can be rapidly discharged through the circuit containing the electrolytic cell. This passage of current takes place in the course of about a few milliseconds. Accordingly, in the appended claims, the term "instantaneous" is employed to describe the brief passage of time during which the current from the external source of direct current is passing through the circuit. Other equivalent means will also be obvious to those skilled in the art. The polarization detector may be a vacuum tube voltmeter or any other suitable means which will quickly recover from the high voltage to which it is initially subjected, and is sensitive to the small differences in electrode potential which are produced in the process. Similarly, any meter which is responsive to the output of the polarization detector may also be employed. In a preferred embodiment, a high speed recorder may be employed to graphically meter the changes in relative potential occurring during the short period of time required to depolarize the test electrodes. As an example of a suitable high speed recorder is a commercially available instrument which was used in this investigation. This apparatus was a strip chart potentiometer recorder having a range of 0-10 millivolts, a 1.5 second full scale balancing time, and a chart speed of about 2 inches per minute. Another means for automatically metering and recording the signal from the polarization detector would be to employ an oscilloscope which was adapted to correlate the polarization-depolarization with time in place of the high speed recorder described in the foregoing embodiment. Thus, by mounting a sensitized photographic plate or paper on the face of the oscilloscope and exposing it to the variations in position of the electron beam caused by subjecting the electron beam to both the cathodic and anodic polarization-depolarization effect, there would be traced a suitable graphical representation of this effect. While a true picture may be obtained with the oscilloscope, there are however certain practical advantages in using a high speed strip chart

recorder to record the phenomena. In addition to the high speed strip recorder and the oscilloscope, a sensitive ammeter may also be employed. While an apparatus employing this expedient would permit the invention to be carried out in a less convenient manner than by means of the apparatus previously described, it is however possible to produce a graphical representation of the algebraic summation of cathodic and anodic depolarization. In employing the apparatus so modified, a sensitive ammeter is connected in the output circuit of a vacuum tube voltmeter. The vacuum tube voltmeter circuit is designed to prevent the power supply voltage from damaging the sensitive meter. The effect of the polarization influences the flow of current in the output circuit of the polarization detector and, as a result, the polarization is made visibly manifest. Inasmuch as the potential difference between two electrodes is correlated with time, the current flow in the polarization output circuit produced by the polarization is visually observed and recorded as though occurring at zero time. The subsequent variation in current resulting from the depolarization is also visually observed and recorded at various time increments until the test electrode potentials return to their normal potential. Cathodic and anodic polarization-depolarization effects are both observed and recorded in this manner, and the data thus obtained are employed to construct a graphical presentation of this effect.

In employing the apparatus of this invention to investigate the rate of corrosion of a metallic material of construction which is exposed to galvanic corrosion, test electrodes 16 and 17 are prepared from the metal which is being studied. These electrodes are substantially identical. It has been found that small diameter rods may be used, however small rectangular coupons are also suitable. After the electrodes have been cleaned and polished, they are placed in the cell 15, which has been filled with an electrolyte which simulates the corrosive environment with which the metal would normally be in contact. The galvanic cell thus prepared is left to stand for about 10 minutes because this time is usually required for reproducible results. After 10 minutes, a composite depolarization curve is obtained by the following procedure: The capacitor 11 is charged by connecting it with the source of high voltage direct current 10. The charged capacitor is then connected between the electrodes 16 and 17 by suitably manipulating the current discharge mechanism. As a result, an instantaneous flow of current is produced across the electrodes by the discharging of the capacitor. The full power supply voltage does not show up on the recorder because the discharge is practically complete by the time the recorder pen has moved a short distance. The variations in electrode potential which are thus produced at both the anode and the cathode are simultaneously detected by the polarization detector and recorded on the polarization meter as a net potential. During the remaining depolarization the changes in electrode potential being produced at the anode and the cathode are simultaneously also detected and the algebraic sum of the variations in potential recorded. The electrodes 16 and 17 are so arranged that the current from the current discharge mechanism flows from one to the other, thus making one electrode cathodic and the other anodic. When no current flows and under normal non-polarized conditions the electrode potential of both electrodes is the same, the difference in potential between them is zero. However when current of sufficient intensity to effect polarization flows between the electrodes, they become polarized and a potential difference appears. The potential difference which is detected is the algebraic sum of the resultant cathodic and anodic polarization. By graphically recording the variations in potential occurring during the polarization-depolarization cycle, there is produced a single composite curve which is a plot of the variation of the algebraic sum of cathodic and anodic polarization

with respect to time. Since depolarization is occurring at the surface of both electrodes, this composite curve is a depolarization-time curve.

It has been found that a correlation exists between the corrosion rate of metals exposed to electrochemical corrosion and the configuration of the depolarization-time curve. It is evident that the slope of the depolarization-time curve should be the basis of the correlation. Possible criteria which may be employed in correlating corrosion rate are, (1) amount of polarization remaining after a given time, (2) difference between polarization voltages at two fixed times, and (3) time required to depolarize to a certain fraction of the maximum recorded polarization. These are illustrative of possible criteria which might be used to correlate the slope of the depolarization-time curve with corrosion rate. Others however will be evident to those who are skilled in this particular art and are also considered within the scope of this invention.

For the purposes of illustrating the instant invention, rate of corrosion of steel exposed to brine solutions was investigated and it was found that in this instance a correlation existed between the corrosion rate and the time required to depolarize to two-thirds of the maximum recorded polarization. This factor will hereinafter be referred to as  $\phi$  and is shown on Fig. 2 in this manner. The fraction  $\frac{2}{3}$  was chosen arbitrarily as being most suitable for this investigation. However, in the event that other corrosive environments are studied, the slopes of the depolarization-time curves should be examined to determine whether or not some other fraction might provide a better degree of correlation. In developing a correlation from polarization data, a series of brine solutions were made up which contained different inhibitors in order that the corrosion rate could be varied. Steel coupons of known weight were suspended in the solution in order to obtain actual weight loss data. These coupons, although immersed in the electrolyte, did not form a part of the polarization measurement system. Electrodes having substantially the same composition as the steel coupons were employed in the same solution to provide the polarization data. As a representative brine, a synthetic aqueous solution was prepared by dissolving 1.95 weight percent NaCl plus 0.49 weight percent  $MgCl_2 \cdot 6H_2O$  in distilled water. This brine solution was air blown until saturated, the oxygen content of the brine then being 6.0 mg./l. Equal portions of this brine were placed in a plurality of beakers and 0.3 percent by weight of inhibitor was added to several of the beakers. Using these solutions as the electrolyte, the above described polarization experiments were conducted using a 100 microfarad condenser charged at 380 volts of direct current and graphical representations of the resulting polarization-depolarization phenomena, as illustrated by Figure 2, were obtained.

The foregoing operating data are only illustrative and non-limiting. In carrying out the instant invention the current density employed in the cell 15 is an important operating variable. It should be sufficient to cause measurable polarization but not high enough to cause a spark discharge across the electrodes 16 and 17 within the cell 15. I have found that the potential of the capacitor or other source of potential should be chosen so that an initial current density of from about 0.03 to 30 amp./cm.<sup>2</sup> is produced, although in some instances current densities outside this range may be used. The time needed to obtain the composite anodic and cathodic polarization-depolarization curve is ordinarily 3 to 5 minutes. This represents the maximum time required. Accordingly, shorter times may be used in some cases.

It is well known that the corrosion rate of steel in aerated brine may change with time. The polarization data should give instantaneous readings, that is, they should tell how fast the metal is corroding while the curve is being obtained. This means that in order to get an accurate correlation, the weight loss data would have

to be obtained over a very short time interval. This procedure would introduce another source of error, namely, that of measuring very small weight losses. Therefore, in addition to the initial curve, similar data were obtained at several periods throughout the run which lasted about 30 hours and an average  $\phi$  for the period of the run of about 30 hours was obtained. Actual weight loss data were obtained from the steel strips which were immersed in the electrolyte during the run.

A plot of  $\phi$  versus the actual corrosion rate in milligrams per square decimeter per day was made using a semilog scale in order to obtain a linear plot. The actual corrosion rate in milligrams per square decimeter per day will hereinafter be referred to as R. From this plot a linear relationship was computed by the method of least squares and it was found that the following relationship between  $\phi$  and R existed for steel exposed to aerated brine:

$$\log \phi = 1.361 - 0.0110R$$

Table I contains a tabular summary of the data obtained from these experiments:

TABLE I  
Corrosion rate data and polarization data for steel in aerated brine at room temperature

| No. | Inhibitor                                                                                | R,<br>MDD                                                                                                             | $\phi$<br>Sec. | Theor.<br>R,<br>MDD | R<br>Expt.-<br>Theor.,<br>MDD |      |
|-----|------------------------------------------------------------------------------------------|-----------------------------------------------------------------------------------------------------------------------|----------------|---------------------|-------------------------------|------|
| 30  |                                                                                          |                                                                                                                       |                |                     |                               |      |
| 1   | Corrosion Inhibitor A consisting of 92% sodium polyphosphate and 8% sodium ferrocyanide. | 1.2                                                                                                                   | 22.2           | 1.2                 | 0                             |      |
| 2   | NaNO <sub>2</sub>                                                                        | 13.3                                                                                                                  | 17.1           | 11.1                | +2.2                          |      |
| 3   | Na <sub>2</sub> B <sub>4</sub> O <sub>7</sub> ·10H <sub>2</sub> O                        | 16.8                                                                                                                  | 13.7           | 20.0                | -3.2                          |      |
| 35  | 4                                                                                        | Corrosion Inhibitor "B" consisting of 4% dodecylamine, 90% tetradeccylamine, 4% hexadecylamine and 2% octadecylamine. | 21.8           | 13.7                | 20.0                          | +1.8 |
| 5   | Corrosion Inhibitor C                                                                    | 25.2                                                                                                                  | 13.7           | 20.0                | +5.2                          |      |
| 40  | 6                                                                                        | Na <sub>2</sub> CrO <sub>4</sub>                                                                                      | 26.5           | 10.8                | 29.0                          | -2.4 |
| 7   | Blank                                                                                    | 32.7                                                                                                                  | 8.8            | 37.0                | +0.7                          |      |
| 8   | Corrosion Inhibitor D                                                                    | 87.0                                                                                                                  | 2.8            | 83                  | +4.0                          |      |

By referring to Table I it is seen that the experimental corrosion rates and the theoretical corrosion rates, as determined by the instant invention, are substantially in agreement. This demonstrates the validity of this correlation and permits an accurate quantitative estimation of the polarization data from corrosion rate.

As it has been pointed out, different corrosive environments in contact with other metallic materials of construction subject to corrosion would produce other empirical relationships because of different corrosion mechanisms. For example, if in the foregoing illustrative description of the invention, oxygen-free brine were employed, the empirical relationship set forth above would probably not hold. In order to develop relationships which are applicable to different environments and different materials, it simply would be necessary to carry out the procedure as outlined above and correlate one aspect of the slope of the depolarization-time curve with the corrosion rate to develop the necessary relationship.

It is thus seen that a quantitative correlation can be established between polarization data and corrosion rate. An extension of this technique would prove useful in making spot corrosion rate checks in pipelines or other installations which are in contact with a corrosive environment. By installing permanent fittings to which are attached two electrodes, the corrosion rate could be checked at any time by interconnecting the electrodes in an apparatus as described above. The use of this technique avoids the effect of residual polarization caused by employing the same electrode for both anodic and cathodic data as well as eliminating the need for a reference electrode. This latter advantage makes possible the use of a simple, rugged installation which could be in-

serted into pipeline and process systems to permit polarization data to be obtained under field conditions.

It will be understood that all changes or modifications of the examples of the invention herein chosen for the purposes of illustration which do not constitute departure from the spirit and scope of the invention are intended to be covered.

What is claimed is:

1. In a method for determining the corrosion rate of a metallic material of construction exposed to electrochemical corrosion, the steps which comprise passing an "instantaneous" discharge of direct current in an amount sufficient to effect measurable polarization through a circuit containing a pair of substantially identical electrodes, prepared from said metallic material, immersed in an electrolytic solution, one electrode being the positive pole and the other electrode being the negative pole, to polarize said electrodes and measuring and recording with respect to time the variations in potential difference between said electrodes during depolarization of said electrodes.

2. A method for determining the corrosion rate of a metallic material of construction exposed to electrochemical corrosion, which comprises immersing in an electrolytic solution a pair of substantially identical electrodes prepared from said metallic material, one electrode being the positive pole and the other electrode being the negative pole, passing an "instantaneous" discharge of direct current in an amount sufficient to effect measurable polarization of said electrodes through a circuit containing said electrodes to effect the polarization of each electrode, detecting electrically and metering with respect to time the variations in potential difference between said electrodes during the depolarization of said electrodes to produce a composite time-potential curve whereby the corrosion rate of said metallic material in contact with an electrolytic environment substantially similar to the

said electrolytic solution can be correlated with aspects of the slope of said curve.

3. A method in accordance with claim 2 in which said net variations in potential difference are graphically metered.

4. A method in accordance with claim 2 in which a current density of from about 0.03-30 amps. per square centimeter is employed.

5. A method in accordance with claim 2 in which the maximum time required to meter said variations in potential difference is from about 3 to 5 minutes.

6. A method for determining the rate of corrosion of steel in contact with aerated brine which comprises immersing a pair of substantially identical electrodes prepared from said metallic material, one electrode being the positive pole and the other electrode being the negative pole, passing an "instantaneous" discharge of direct current in an amount sufficient to effect measurable polarization of said electrodes through a circuit containing said electrodes to effect the polarization of each electrode, detecting electrically and metering, with respect to time, the variations in potential difference between said electrodes during the depolarization of said electrodes to produce a composite time-potential curve, and determining the time required to depolarize from 50 to 75 percent of the maximum polarization whereby the corrosion rate of steel in contact with aerated brine may be computed from said determined time.

7. A method in accordance with claim 6 in which the said time is the time required to depolarize to about two-thirds of the maximum polarization.

#### References Cited in the file of this patent

"Transactions of The Electrochemical Society," vol. 81  
35 (1942), pages 278-281 of paper by Ferguson et al.

"Corrosion and Material Protection," January 1948,  
30 pages 15-20, paper by Marsh.